

## UNITED STATES PATENT OFFICE

2,120,678

## BLEACHING AND PURIFYING PROCESS

John L. Parsons and Donald T. Jackson, Erie,  
Pa., assignors to Hammermill Paper Company,  
Erie, Pa., a corporation of Pennsylvania

No Drawing. Application March 30, 1936,  
Serial No. 71,690

8 Claims. (Cl. 8—108)

This invention relates to an improved bleaching and purifying process particularly adapted for the bleaching and purification of cellulose fibers derived from wood or the like by any of the known fiber-liberation processes. While it is capable of general application to pulps of all types, it is especially suited for the treatment of 5 kraft or sulfate pulps. The resulting product is excellently suited for use in the paper industry and in the rayon, film, and similar industries.

Kraft or sulfate pulps have always presented a difficult problem in the matter of bleaching to a satisfactory white color. If an attempt is made to bleach such pulps by the ordinary hypochlorite treatment, used extensively in connection with sulfite pulp, serious injury will be done to the fibers before they are brought to a satisfactory color for use in white paper stock. This is due to the excessive amount of the hypochlorite required to produce the desired result. We have discovered, however, that kraft or sulfate pulp may be bleached to a high white color without serious injury to the fibers through the proper use of a chlorite in lieu of part or all of the hypochlorites ordinarily employed. In fact, through 15 the use of a three-stage process, one stage of which involves a chlorite treatment, the strength of the bleached and purified product will be equivalent or superior to that of the unbleached pulp. Other improvements will also be noted. In attempting to bleach and purify pulp by the 20 usual methods, new impurities in the form of degraded cellulose are produced. Such new impurities are not produced, however, in the practice of the present improved process.

The three-stage process referred to involves a preliminary treatment of the pulp with free chlorine. While such a treatment alone is quite 25 unsatisfactory for producing a pulp of high white character, especially kraft pulp, it will be found to pave the way excellently for the chlorite treatment which follows. Between the chlorine and the chlorite treatments there is preferably, though not necessarily, added to the pulp a sufficient quantity of any suitable alkali to react with all of the available chlorine and the pulp is then washed. In reacting with the chlorine the alkali will form a hypochlorite which in turn will quickly be consumed in reaction with the pulp. The 30 alkali also reacts directly with certain impurities

in the pulp, largely produced by the chlorination, and renders these impurities soluble. If desired the alkali treatment may be preceded as well as followed by a washing of the pulp and it may be extended over a considerable period, say an hour or even more. Following the chlorite treatment, which will be described in greater detail herein-after, the pulp is again washed and then a relatively small amount of calcium or sodium hypochlorite or the like is added to complete the 10 bleach. In many cases a satisfactory whiteness will be attained without the final hypochlorite treatment or by substituting for it a second chlorite treatment. Excellent results have been obtained by the use of a mixture of a chlorite with 15 hypochlorite following the chlorine treatment or as the final treatment of the pulp following a treatment with a chlorite alone. Also in many cases, particularly when dealing with sulfite and soda pulps, very good results may be obtained 20 without the preliminary chlorine treatment, in which case the process will preferably involve a chlorite treatment followed by a hypochlorite treatment.

Inasmuch as the chlorite treatment forms the 25 most important feature of the improved process the preferred manner of carrying it out will now be described in some detail. We have found sodium chlorite to be especially suited for the purposes of this stage of the process although many 30 other chlorites might also be used, particularly the chlorites of the alkali and alkaline-earth metals and also ammonium chlorite. The quantity of the chlorite to be used depends upon the character of the other steps of the process. Ordinarily the bleaching of a particular type of pulp to a particular state of whiteness will require a certain amount of available chlorine. The precise amount of available chlorine to be supplied through the chlorite will depend upon how much, 35 if any, is supplied in the form of free chlorine and how much, if any, is supplied through a hypochlorite. Sulfite pulps will usually require between 2.5 and 6.5% available chlorine (based upon the weight of the dry fiber in the pulp) to 40 effect a thorough bleaching. Kraft pulp on the other hand will require in the neighborhood of 15% available chlorine on the same basis. Very good results are obtainable through the use of 45 sufficient of the chlorite to provide about one- 50

fourth of the total available chlorine used. This may readily be varied, however, according to circumstances so that anywhere from 10 to 50% or more of the total available chlorine is provided 5 through the chlorite.

In treating the stock with a chlorite we have employed pulp consistencies of 5 to 10 per cent. If desired the consistency might be made lower, e. g. 1 or 2%, but this will entail additional expense due to the greater bulk of the equipment required, the greater input of heat required, and various other considerations. In general it is preferable to employ higher consistencies and, if the equipment available for the handling of the 10 stock is appropriate, much higher consistencies may be employed. In fact consistencies of as much as 20 to 30% or even more may then be utilized.

The chlorite treatment should be carried out 20 in or with a solution that is on the acid side and preferably one that has a pH value of about 4.0. At this degree of acidity the reaction will take place at a relatively rapid rate with very satisfactory results. However, good results may be 25 obtained at any pH between 3.0 and 6.0. At the higher pH values the reaction becomes somewhat slower while at a pH below 3.0 there is a tendency for the chlorites to decompose rather rapidly. During the course of the chlorite treatment 30 the solution has a tendency to become more strongly acid, i. e. if it starts with a pH of 4.0 it will conclude with a pH around 3.5. For the purpose of establishing the desired acidity a suitable quantity of any appropriate acid, such 35 as hydrochloric or sulfuric acid, may be added. Hydrochloric acid is preferred, due to the soluble salts formed and its strength, but a variety of other acids, particularly the mineral acids, might be used.

40 For best results the mass should be heated to a temperature of about 50° C. for the chlorite treatment. The reaction is considerably more rapid at a slightly elevated temperature of this character than at ordinary room temperatures. 45 However, if the acidity of the mixture is sufficiently great a reasonable rapid reaction will take place at ordinary temperatures of around 20° C. On the other hand, so long as the acidity is not too great, i. e. not below a pH of about 4.0, the temperature may well be carried up to 50 60° C., or even higher. Above 60° C. at a pH of 4.0 the decomposition of the chlorite will become objectionably rapid but if the pH is higher the temperature may be correspondingly higher 55 without too rapid decomposition of the chlorite. Accordingly the temperature may well be varied between 20° and 60° C., or even broader limits, depending upon the other conditions prevailing.

A typical operation of a three stage process 60 conducted in accordance with the invention will now be described. A sulfite pulp requiring about 3.5 per cent available chlorine, based on the weight of oven dry pulp, to produce a satisfactory white color when bleached with calcium hypochlorite in a single stage process was subjected to the following treatments: For the first stage sufficient chlorine, in the form of chlorine water, was added to provide 2% of available chlorine, based upon the weight of the oven dry fiber. 65 The pulp suspension during this treatment was 70 suitably maintained at a consistency of 3 per cent and at a temperature of about 22° C. After six minutes of this treatment, during which the stock was agitated continuously, there was added 75 a sufficient quantity of an alkali to consume all

of the remaining available chlorine and furnish an alkaline solution. For this purpose 2.4% of calcium hydroxide, based on the weight of the dry pulp, was found sufficient. Corresponding amounts of other alkalis such as sodium hydroxide, potassium hydroxide, or ammonium hydroxide or in fact any hydroxide of the alkali and alkaline-earth metals, or carbonates of the alkali metals, might have been substituted for a part or all of the calcium hydroxide. Following the 10 addition of alkali the pulp was washed and it was then ready for the second stage of chlorite treatment. In preparation for this it was first reduced to a consistency of 5% and was then heated to a temperature of about 50° C. Prior to the 15 heating a sufficient quantity of sodium chlorite was added to provide available chlorine to the extent of .75% of the weight of the dry pulp and sufficient hydrochloric acid was added to bring about a pH value of 4.0. This chlorite treatment 20 was continued for a period of three and three quarters hours during which the mass was agitated continuously. At the conclusion of this treatment the pulp was thoroughly washed and then reduced again to a 5% consistency preparatory 25 to the third stage treatment. In the third stage sufficient calcium hypochlorite was added to provide an available chlorine content of 0.40 per cent of the weight of the dry fiber. The temperature during this stage in the typical operation 30 was maintained at about 38° C. After a period of two hours, during which the pulp was continuously agitated, the bleached material was again thoroughly washed.

The product resulting from the foregoing three 35 stage treatment exhibited properties different from and superior to the products of prior known bleaching processes. One startling characteristic of the new bleached product was that paper produced from it had a greater folding endurance, 40 by the Schopper test, than paper of the same weight and character produced from the unbleached sulfite pulp. Thus the paper formed from the new product displayed a folding endurance of 1170 while paper formed from the 45 same stock prior to bleaching displayed a folding endurance of only 910. This is quite remarkable inasmuch as paper formed from the same stock bleached by a two stage, chlorine and hypochlorite, process developed a folding endurance 50 of only 680. This is the ordinary experience, i. e. prior bleaching processes have tended to reduce the folding endurance of the stock greatly while the product of our new process has an increased folding endurance, as compared with the original 55 unbleached stock. In the determination of the values given above, standard methods and equipment were employed in connection with 20 lbs. basis weight sheets, (17" x 22"—500 sheets).

So also from the standpoint of strength, as determined by the standard Mullen bursting strength test applied to the same 20 lb. basis weight sheets, the new product is superior to the product of prior known bleaching processes. Paper formed in the standard way from the new 65 bleached product has a Mullen bursting strength of 52 as compared with a strength of 53 for the unbleached sulfite pulp and 50 for the same pulp bleached by a two stage chlorine-hypochlorite process. The foregoing physical tests were conducted at a temperature of 70° F. and a relative 70 humidity of 50%.

The following table giving a comparison of the results obtained in certain tests upon the raw, unbleached sulfite pulp of the typical example, the 75

bleached product of the typical example, and the same initial stock subjected to a two stage, chlorine-hypochlorite bleaching process, discloses the superiority of the new process and product in the foregoing and other respects:

|                                    | Un-bleached pulp                                                          | Three stage bleaching using chlorite | Two stage chlorine hypochlorite bleached |
|------------------------------------|---------------------------------------------------------------------------|--------------------------------------|------------------------------------------|
| 10                                 |                                                                           |                                      |                                          |
| Total percent av. Cl, added        |                                                                           | 3.15                                 | 2.75                                     |
| Total percent av. Cl, consumed     |                                                                           | 2.85                                 | 2.61                                     |
| Bursting strength (Mullen)         | 53                                                                        | 52                                   | 50                                       |
| 15                                 | Folding endurance (Schopper)                                              | 910                                  | 1170                                     |
| Viscosity in cuprammonium solution | 69                                                                        | 47                                   | 32                                       |
| Percent alpha cellulose            | 85.5                                                                      | 85.8                                 | 85.4                                     |
| Copper number                      | 1.7                                                                       | 1.4                                  | 1.3                                      |
| Percent hot alkali soluble         | 20.9                                                                      | 19.6                                 | 21.9                                     |
| 20                                 | Brightness (percent reflectance with #1 filter in G. E. reflection meter) | 59                                   | 90                                       |
|                                    |                                                                           |                                      | 87                                       |

In the foregoing the viscosity in cuprammonium solution and the alpha cellulose content have been determined according to the methods adopted by the Technical Association of the Pulp and Paper Industry. The copper number has been determined by the Schwalbe-Hägglund method and the "per cent hot alkali soluble" has been determined by the Lynch method as outlined in Industrial Engineering Chemistry 22, 952-3/1930. In another typical operation in accordance with the invention a Swedish kraft pulp was subjected to a three stage treatment of the same general character as specified in the first example except that the quantities of the various treating agents were greatly increased and the chlorine treatment extended over a period of 45 minutes after which the pulp was washed and then treated with 0.5 per cent of calcium hydroxide, based on the dry pulp weight. In the first stage sufficient chlorine was consumed to constitute 7.66% based upon the weight of the dry fiber. In the next stage sufficient sodium chlorite was consumed to provide available chlorine to the extent of 5.96% of the dry pulp weight, while in the final stage sufficient calcium hypochlorite to provide 0.85% available chlorine was consumed. Tests of the same character as outlined above, together with a standard (Thwing) tearing test applied to 20 lb. basis weight paper (17" x 22" - 500 sheets) at 50% relative humidity and 70° F., gave the following results:

|                                                                           | Un-bleached pulp                   | Three stage bleaching using chlorite |    |
|---------------------------------------------------------------------------|------------------------------------|--------------------------------------|----|
| 55                                                                        |                                    |                                      |    |
| Bursting strength (Mullen)                                                | 61                                 | 65                                   |    |
| Folding endurance (Schopper)                                              | 1630                               | 1800                                 |    |
| Tearing (Thwing)                                                          | 93                                 | 104                                  |    |
| 60                                                                        | Viscosity in cuprammonium solution | 112                                  | 30 |
| Brightness (percent reflectance with #1 filter in G. E. reflection meter) | 25                                 | 83                                   |    |

From the foregoing it will be seen that the bleached kraft resulting from the improved process not only displayed greater folding endurance but also better strength and better tear resistance than the initial, unbleached stock. This is directly contrary to the usual experience with products of other bleaching processes. Furthermore, this is in spite of the fact that the kraft pulp was bleached to an exceptionally high, white color. The high viscosity of the highly bleached product is also noteworthy. It is desirable for various purposes to maintain the viscosity value specified as high as possible, preferably over 25, but

prior bleaching processes in dealing with kraft or sulfate pulp have failed to achieve this end. It has not been considered possible, heretofore, to combine high strength, high viscosity and a high white color in a kraft or sulfate pulp product.

While the preferred three stage process has been described in considerable detail it will be understood that wide latitude is permissible in the practice of the invention. The preliminary chlorine treatment may be carried out in any known manner and may provide any desired portion of the total available chlorine used. Preferably 50% of more of the total available chlorine is supplied in this way but, if preferred, only 25% of the total need be so supplied. Furthermore, good results can be obtained with sulfite pulp if the chlorine treatment is omitted altogether in which case the process will preferably consist of one or two chlorite treatments followed by a hypochlorite treatment. The permissible latitude in the chlorite treatment has already been referred to. While it is preferred to conclude the three stage process with a hypochlorite treatment of any suitable character, this is not essential and the hypochlorite may be replaced by a second chlorite treatment. When the hypochlorite is used it should preferably supply only about 5 to 15% of the total available chlorine consumed. Should the preliminary chlorine treatment be omitted, however, a somewhat greater quantity of hypochlorite may be employed, to supply, say up to 35% of the total required available chlorine. If desired the chlorite and hypochlorite treatments may be combined into a single stage or treatment with a chlorite alone may be followed by a treatment with a mixture of a chlorite and a hypochlorite. In any case the combined available chlorine should be substantially as specified and preferably the relative proportions of chlorite and hypochlorite should be as stated, although when a mixture is used the chlorite and hypochlorite may, if desired, be present in about equal proportions. When the mixture is used the temperature of the stock may suitably be maintained around 35 to 40° C. and the pH at between 7 and 9 although these conditions may be varied to suit the particular circumstances. When the chlorite predominates in the mixture the conditions should approach more nearly those preferred for the chlorite treatment alone. It will be understood that appropriate washing and alkali treatments will be employed whether the chlorine treatment is followed by separate chlorite and hypochlorite treatments or by treatment with a mixture. The duration of the various stages of the process will depend upon the amount of available chlorine supplied in each stage and upon the temperature and other operating conditions. The periods specified under the typical example have been found quite satisfactory for the conditions mentioned.

The terms and expressions used herein are to be regarded as terms of description and not of limitation.

What is claimed is:

1. A method of bleaching and purifying cellulosic material which comprises first subjecting the cellulosic material to the action of chlorine, then treating the same with a chlorite selected from the class consisting of an alkali metal and an alkaline earth metal, and finally subjecting the cellulosic material to the action of an alkaline hypochlorite.

2. A method of bleaching and purifying cellulosic material which comprises subjecting the same in a plurality of stages to the action of a plurality of agents having available chlorine, at least one of said agents being in the form of a chlorite selected from the class consisting of an alkali metal and an alkaline earth metal, and another of said agents being in the form of a hypochlorite, the final stage comprising treatment with an alkaline hypochlorite.
3. A method of bleaching and purifying cellulosic material which comprises successively subjecting the same to the action of chlorine, a chlorite selected from the class consisting of an alkali metal and an alkaline earth metal, and a hypochlorite, in the sequence specified, the chlorite treatment being conducted in the acid state at a temperature of about 50° C. and the hypochlorite treatment being conducted in the alkaline state at a temperature of about 38° C.
4. A method of bleaching and purifying cellulosic material which comprises successively subjecting the same to the action of chlorine, sodium chlorite, and calcium hypochlorite in the sequence specified, said hypochlorite being in alkaline solution.
5. A method of bleaching and purifying cellulosic material which comprises subjecting the same to the action of chlorine and then subjecting it to the action of a mixture of a chlorite and a hypochlorite.
6. A method of bleaching and purifying cellulosic material which comprises subjecting the same to the action of a mixture of a chlorite and a hypochlorite at a pH of at least 7.0.
7. A method of bleaching and purifying cellulosic material which comprises subjecting the material to the action of chlorine, a chlorite and a hypochlorite in a plurality of stages, the hypochlorite being used at least in part in the final stage and in a quantity to provide available chlorine to the extent of not more than 1% of the dry weight of the material being bleached, said final stage being carried out in alkaline solution.
8. A method of bleaching and purifying cellulosic material which comprises subjecting the same in a plurality of stages to the action of a plurality of agents having available chlorine, at least one of said agents being in the form of a chlorite and providing from 10 to 50% of the available chlorine consumed, and another of said agents being a hypochlorite and providing from 5 to 35% of the available chlorine consumed, said hypochlorite being used in an alkaline state in the final bleaching stage.

JOHN L. PARSONS.  
DONALD T. JACKSON.